

## UNITED STATES PATENT OFFICE

2,035,742

## PURIFICATION OF NAPHTHENIC ACIDS

Frederick J. Ewing, Pasadena, Calif., assignor to  
 Union Oil Company of California, Los Angeles,  
 Calif., a corporation of California

No Drawing. Application March 12, 1934,  
 Serial No. 715,181

22 Claims. (Cl. 260—108)

This invention relates to naphthenic acids and more particularly refers to a process for their deodorization and decoloration.

It is an object of my invention to present a simple, efficient and thoroughly satisfactory process for obtaining naphthenic acids of a light color and bland odor.

Naphthenic acids, such as may be obtained by acidifying various alkaline liquors arising during the refining of petroleum or shale oil fractions, constitute a complex mixture of acidic compounds containing principally carbon, hydrogen and oxygen. They range from comparatively low-boiling liquids to materials which are solid or semi-solid at ordinary temperatures. Their viscosities as well as their boiling points are generally closely correlated to the viscosities and boiling points of the hydrocarbon fractions in which they are present.

The crude naphthenic acids which are obtained by acidifying the alkaline liquors referred to above, contain varying amounts of phenols and carbonaceous materials and they possess a very dark to black color and a disagreeable odor. When these crude acids are freed from phenolic materials by careful acidification, neutralization and distillation as hereinafter described to produce what will hereinafter be called "semi-refined" acids, the amount of carbonaceous materials appears to increase as a result of which 3 to 5% thereof and sometimes even greater amounts have been encountered in the dephenolized naphthenic acids. The major portion of this carbonaceous material is present in a finely suspended or colloidal state and is in most instances not removable by settling or centrifuging. The presence of this material is partially responsible for the dark and turbid color of the naphthenic acids and renders their sale as a commercial product practically impossible. It is, therefore, desirable to obtain naphthenic acids which are substantially free from these undesirable materials.

It has been customary to distill the naphthenic acids to remove this carbonaceous material. However, this distillation is not applicable in all instances in that it is usually accompanied by plugging of the still due to the presence of the aforementioned carbonaceous material. Moreover, the equipment used for this distillation is subject to a rapid deterioration due to the corrosive action of the naphthenic acids on iron or on other metals normally used in the construction of stills. The naphthenic acids which are recovered as an overhead product of such a distillation are of a substantially improved color, but this color on stand-

ing rapidly darkens and in some instances becomes nearly as dark as before distillation.

A more efficient and satisfactory method for removing this carbonaceous material consists in treating the crude or semi-refined naphthenic acids with any of the common oxygen-containing inorganic acids, such as sulphuric acid of suitable concentration, whereby a coagulation and separation of this carbonaceous material is brought about. The product obtained by this method of treatment which will be described in greater detail later on, is of a somewhat improved color but still is inapplicable without further treatment in any instances where a light colored product is desired.

I have discovered that naphthenic acids from which the carbonaceous materials have been removed by either of the two above identified processes or by any other physical or chemical means such as those hereinafter set forth, may be worked up into a product of excellent light color which does not change or darken on exposure, and bland odor, by treating them subsequently to the removal of the carbonaceous materials with an adsorbent material such as clay, fuller's earth, "Filtrol" or activated carbon. By so operating, a distillation of the naphthenic acids to bring about a further improvement in color and odor may be eliminated. This treatment with adsorbent materials is substantially ineffective where the carbonaceous materials have not been previously removed. However, the acid treatment of the naphthenic acids for purposes of removing the carbonaceous materials renders them especially suitable for further purification by means of the adsorbent.

While it is customary to remove the residual inorganic acidity from the naphthenic acids which have been treated with an oxygen-containing inorganic acid such as sulphuric acid for the removal of the admixed carbonaceous materials, experiments have indicated that the treatment with the adsorbent material may be substantially improved by eliminating the water wash for the removal of this inorganic acidity, and contacting the naphthenic acids with the adsorbent material in the presence of small amounts of an inorganic acid thus remaining in the naphthenic acids. As a slight modification of the above method of treatment, I may activate the clay or other adsorbent with small amounts of sulphuric acid or any of the other acids set forth herein by adding these acids to the adsorbent and treating the naphthenic acids with the mixture of adsorbent and acid. Activation of the clay with

acid salts, i. e. a salt which on solution liberates hydrogen ion, produces substantially identical results as in the case where an inorganic acid is used for activating the adsorbent. If desired,

5 I may also add my inorganic acid directly to the naphthenic acids before adding the adsorbent material, whereby the same effect of activation of the adsorbent is obtained.

Therefore, my invention broadly resides in a 10 process for obtaining naphthenic acids of a stable light color and bland odor which comprises removing the carbonaceous material present in these acids and subsequently treating the product so obtained by means of an adsorbing agent.

15 My invention likewise extends to a process for purifying and decolorizing naphthenic acids wherein the adsorbing agent used has been activated or treated with an inorganic acid such as sulphuric acid or with an acid salt such as sodium 20 acid sulphate or sodium acid phosphate or the like.

The term "alkaline liquor" referred to earlier in this specification relates not only to the alkaline solution containing naphthenic acids and 25 other materials taken up by the alkali on treating a petroleum fraction but also relates to the alkaline solution obtained by treating the extract phase which is formed on treating a petroleum fraction with a selective solvent such as liquid 30 sulphur dioxide, dichlorethyl ether, nitrobenzene, furfural, isopropyl alcohol, dimethyl sulphate, etc., with caustic soda, caustic potash or any other alkaline reagent.

When an alkaline liquor, arising on treatment 35 of petroleum fractions such as any of those described above, is acidified with any of the well known inorganic acids a distinct phase separates out which phase is then adjusted by means of sodium carbonate or sodium hydroxide (or their 40 equivalents) to a pH of about 9. By so operating there is formed a mixture consisting of sodium naphthenates, phenols and admixed hydrocarbons which is then subjected to distillation which removes the phenols and hydrocarbons overhead. 45 The still bottoms then consist of sodium naphthenates, which, when dissolved in water form a solution from which the semi-refined acids are obtained by the addition of a mineral acid such as sulphuric acid.

50 These semi-refined naphthenic acids contain from 3 to 5% of carbonaceous material, only a small fraction of which is removable by settling or centrifuging. Apparently this material is present in some kind of colloidal suspension 55 which renders its separation extremely difficult. In addition, they are of a red to dark black color rendering their use as a commercial product practically impossible.

In a co-pending application, Serial No. 696,914, 60 there is set forth a process for removing carbonaceous materials from, crude or semi-refined naphthenic acids which process, in its simplest aspect, relates to the treatment of naphthenic acids with oxygen-containing inorganic acids of 65 such concentration that the formation of emulsions is substantially prevented and a ready separation of the sludge formed upon acid treatment may be realized. For instance, sulphuric acid, having a concentration between approximately 70 50 and 83% has been found especially suitable. While any oxygen-containing inorganic acid such as iodic acid, chloric acid or bromic acid has been disclosed as suitable for the separation of the carbonaceous materials, we preferably use an 75 oxygen-containing inorganic acid chosen from

the class comprising sulphuric, phosphoric or nitric acid. The amounts of these acids to be used are relatively small and range from  $\frac{1}{2}$  to 10 volume percent of the naphthenic acids.

If desired, the acid treatment referred to above, 5 may be carried out in the presence of a hydrocarbon diluent such as liquid propane, butane, cleaner's naphtha (a petroleum fraction boiling between 200-300° F.) benzol or the like. The addition of any of the above mentioned diluents 10 greatly facilitates the separation of the sludge formed as a result of the acid treatment.

I have discovered in connection with the present invention that a similar facilitation of the sludge settling may be brought about by increasing 15 the temperature of the acid treatment to temperatures ranging from approximately 100 to 200° F.

While in the above identified application it is indicated that the strength of the acid used for 20 the removal of the carbonaceous materials should preferably be between 50 and 83%, I have found that acids of greater concentration may be used as well and that such acids are especially effective when a naphthenic acid product of light 25 color is desired. As such concentrated acids are more or less miscible with the naphthenic acids, steps must be taken to provide for the removal of these acids as well as for the acid sludge. Thus 30 95% sulphuric acid, fuming sulphuric acid (containing about 15% dissolved  $\text{SO}_3$ ) as well as sulphuric acid having a concentration of between 83 and 95%, tend to be substantially miscible with the naphthenic acids.

When the impure naphthenic acids containing 35 carbonaceous materials are contacted with  $\frac{1}{2}$  to 10 volume percent of sulphuric acid having a concentration substantially that set out above, no separation into phases takes place, although 40 in some cases the carbonaceous materials agglomerate. However, when portions of more dilute sulphuric acid (e. g. sulphuric acid of 60% concentration) are added to the mixture of impure naphthenic acids and the highly concentrated sulphuric acid, a separation into a naphthenic acid phase and a phase consisting of 45 sludge, sulphuric acid and carbonaceous materials readily takes place as soon as the total acid concentration has been reduced to approximately 83%. The carbonaceous materials are found in 50 the sludge and sulphuric acid layer.

Another method of obtaining phase separation when such concentrated acids are being used to obtain a higher degree of decolorization and deodorization consists in diluting the naphthenic acids either before or after treatment with the concentrated sulphuric acid, with a material capable of reducing the solvent power of the sulphuric acid for the naphthenic acids. Liquid propane, cleaners' naphtha, petroleum ether or other 60 light paraffinic solvents may be used for this purpose. Aromatic hydrocarbons, such as benzol, toluol or their homologues may be used for the purpose indicated above but are not as desirable 65 as the paraffinic solvents on account of their solubility in the concentrated sulphuric acid. The above mentioned diluents may be removed from the naphthenic acids by distillation or by extracting the mixture of naphthenic acids and diluent with an alkaline material, such as caustic soda and liberating the naphthenic acids from their salts so produced by means of an inorganic acid such as  $\text{H}_2\text{SO}_4$ ,  $\text{HCl}$  or the like.

70 The so treated acids are then treated with the 75

adsorbent material in the manner described herein, to further improve their color and odor.

When the crude or semi-refined naphthenic acids, before subjecting them to the above mentioned acid treatment are contacted with an adsorbent material while agitating the mixture either by air or by mechanical means, no improvement in color or odor of the naphthenic acids is brought about after filtering off the latter from the adsorbent. Even in the case where the naphthenic acids and adsorbent were heated to temperatures substantially in excess of atmospheric, no improvement in the color thereof could be noted.

When, however, the carbonaceous materials are removed from the naphthenic acids by means of any of the oxygen-containing inorganic acids set forth in the above identified co-pending application or by any other means and the so treated acids are subjected to a treatment with an adsorbent material a vast improvement in the color and odor of the final product as compared with the crude or semi-refined acids is brought about.

For example, in a preliminary experiment, impure naphthenic acids which had been treated with 0.5% by volume of 80% sulphuric acid for purposes of removing the carbonaceous materials admixed therewith, and which had a color in excess of 8 N. P. A., were contacted with 10% of fuller's earth for 5 minutes at a temperature of 300° F. After filtering off the adsorbent and the materials taken up thereby, naphthenic acids having a color of from 4 1/4 to 5 1/4 N. P. A. was obtained. The same acids, without preliminary acid treatment, when contacted with the same adsorbent under identical conditions showed no improvement in color whatsoever.

Considering my process in greater detail, a charge of crude or semi-refined naphthenic acids contaminated with carbonaceous materials and having a dark red to black color, is treated with an oxygen-containing inorganic acid such as sulphuric acid. The amount of acid used may vary between 1/2 to 10 volume percent of the naphthenic acids. The concentration thereof is chosen preferably between 50 and 83%. The mixture of inorganic acid and naphthenic acids is agitated with air or by mechanical means preferably for a period of from 15 to 30 minutes. Just before the agitation is stopped, a small amount of clay or water is added to facilitate the separation of the acid sludge. The sludge is subsequently separated together with the carbonaceous materials. The naphthenic acids are then washed with water to remove any inorganic acidity and are then blown at a slightly elevated temperature with natural gas or any inert hydrocarbon gas to remove the remaining traces of water.

The naphthenic acids, treated as indicated above, have a much improved color but are still too dark for a commercial product. These acids are now mixed at ordinary temperatures or at least at temperatures below the boiling point of water, with the adsorbent, the amount of the latter being somewhere between approximately 8 and 20%, depending upon the particular charge of the naphthenic acids and the degree of decolorization desired. The mixture of naphthenic acids and adsorbent is heated while agitating with air or by other means, such as a mechanical stirrer up to a temperature ranging from approximately 225° F. to 300° F. or higher. As soon as the desired temperature has been reached, which in most instances is somewhere between 250° F. and 325° F., the heating is discontinued or slowed

down and the mixture is maintained at this temperature for a period of approximately 2 to 5 minutes. The agitation is then discontinued, and the purified and decolorized naphthenic acids are separated from the adsorbent by filtering them while still in a heated condition through a suitable filtering device such as a Sweetland filter. It is not essential that the filtering process takes place at an elevated temperature. However, the viscosity of the naphthenic acids at an elevated temperature is such to allow a more rapid filtration. The naphthenic acids so obtained have a color of from 4 to 6 N. P. A. as compared with a color in excess of 8 N. P. A. before treatment with the adsorbent.

As a slight modification of the above operation, it may be desirable in connection with the purification of the naphthenic acids to eliminate the water wash of the naphthenic acids for removal of the inorganic acidity and thus leave a small amount of sulphuric acid or any equivalent acid, admixed with the naphthenic acids. When the naphthenic acids containing a small amount of inorganic acidity are treated with the adsorbent material a product is obtained which has a lighter color than one which had been water washed before treatment with the adsorbent. It is believed that the presence of the inorganic acid tends to activate the adsorbent material.

If for any reason a water wash of the naphthenic acids should be deemed desirable, the adsorbent may be activated by addition of small amounts of an inorganic acid such as that used for the removal of the carbonaceous materials or these acids may be directly added to the naphthenic acids before treatment with the adsorbent as pointed out above. Acid salts such as sodium acid sulphate, sodium acid phosphate or the like may be substituted for the inorganic acids and produce almost identical results. It has been found advantageous, especially in the case where the residual inorganic acid is used for activating the adsorbent material, to introduce a small amount of water with the adsorbent, or adding the adsorbent in the form of a water containing slurry. The presence of the water appears to cause a better dispersion of the inorganic acid and hence a better activation of the adsorbent material.

The amount of the adsorbent to be used will vary with the naphthenic acid stock to be treated, the degree of decolorization and the particular adsorbent used. In general, amounts of from 8 to 20% of the adsorbent material as indicated above are sufficient, although in certain instances where a light colored product is desired, from 40 to 51% of the adsorbent material may be required.

The treating temperature with the adsorbent material referred to above has been indicated to be somewhere between approximately 225° F. to 325° F. However, very successful treatments have been made at temperatures of 400° F. or above. The above temperature range is merely my preferred operating temperature. Naphthenic acids, freed from carbonaceous materials by any of the processes set forth herein, show an improvement in color even when treated at room temperature. The upper treating temperature limit is largely controlled by the boiling point and flash point of the naphthenic acids.

The time interval during which the naphthenic acids are contacted with the adsorbent material may vary over a wide range. In general, 2 to 15 minutes are sufficient to bring about the desired

decolorization although contact times considerably in excess of these may be necessary in certain instances.

The following specific examples are illustrative 5 of my invention:

*Example 1*

Fifteen hundred (1500) cubic centimeters of semi-refined naphthenic acids containing from 10 3 to 5% of carbonaceous materials were agitated with 75 cubic centimeters of 80% sulphuric acid for one-half hour. Immediately before the agitation was stopped, 5 grams of diatomaceous earth were added to the mixture to facilitate the settling of the sludge. The naphthenic acids, now 15 substantially free from the above mentioned carbonaceous materials, were washed with hot salt water and after removal of the wash water, were

The finished product in each instance had an acid number of from 289-290, as compared with an acid number of 284 before treatment.

The following example is illustrative of the improved decolorizing action of the adsorbent 5 when small amounts of sulphuric acid are left in the naphthenic acids which in this case is accomplished by eliminating the water wash. The stock used consisted of semi-refined naphthenic acids which had been agitated with 5 volume percent of 80%  $H_2SO_4$ . (About 1% of clay was added to facilitate the settling of the sludge.) The results of the treatment of these acids with the adsorbent in comparison with naphthenic acids 10 which had been water washed for removal of the 15 sludge are given below:

*Table II*

| 20 | Type of acids.            | Semi-refined naphthenic acid treated as indicated above | Same           | Same                       | Same           | 20 |
|----|---------------------------|---------------------------------------------------------|----------------|----------------------------|----------------|----|
| 25 | Water wash                | None                                                    | None           | Agitated with 10% $H_2O$ . | Same.          | 25 |
|    | Clay used—amount          | 10% "Filtrol"                                           | 10% "Filtrol"  | 10% "Filtrol"              | 10% "Filtrol". |    |
|    | Clay treating temperature | 200° F.                                                 | 225° F.        | 225° F.                    | 225° F.        |    |
|    | Duration of clay treating | 2 min.                                                  | 2 min.         | 2 min.                     | 2 min.         |    |
| 30 | Color of filtrate         | 4 1/4 N. P. A.                                          | 4 1/4 N. P. A. | 6 1/4 N. P. A.             | 6 1/4 N. P. A. | 30 |

blown bright with natural gas, at a temperature of about 180° F. They were transparent when viewed through the neck of a four ounce oil sample bottle, whereas the untreated acids were black and had no such transparency.

The naphthenic acids which had been purified as indicated above were then mixed at room temperature with approximately 10% by weight of "Filtrol". Individual samples of the mixture 40 were slowly heated up to a temperature of approximately 212° F. to cause a dehydration of the adsorbent in such a manner that no undue foaming of the mass occurred and they were 45 then heated to various temperatures ranging from 225° F. to 300° F. The naphthenic acid charges, during heating, were agitated by means of a slow current of air. When the desired temperature had been reached, the heating of the 50 charges was slowed down or discontinued and the mixture of naphthenic acid and clay was allowed to remain at this temperature for approximately two minutes. The acids were then removed from the adsorbent materials by passing 55 the mixture through a suitable filtering device. This filtration was carried out at substantially the same elevated temperature which prevailed during the clay treatment which greatly facilitated the rate of filtration.

The finished product has a permanent color 60 of from 4 1/4 to 5 1/4 N. P. A. and was of a bland to sweet odor as may be seen from the following table:

*Table I*

| 65 | Stock treated                  | Semi-refined acid        | Semi-refined acid        | Semi-refined acid        | Semi-refined acid        | 65 |
|----|--------------------------------|--------------------------|--------------------------|--------------------------|--------------------------|----|
| 70 | Volume of acid treat           | 5 vol.% of 80% $H_2SO_4$ | 5 vol.% of 80% $H_2SO_4$ | 5 vol.% of 80% $H_2SO_4$ | 5 vol.% of 80% $H_2SO_4$ | 70 |
|    | Adsorbent used                 | "Filtrol"                | "Filtrol"                | "Filtrol"                | "Filtrol"                |    |
|    | Temperature of "Filtrol" treat | 75° F.                   | 225° F.                  | 250° F.                  | 300° F.                  |    |
|    | Duration of "Filtrol" treat    | 2 min.                   | 2 min.                   | 2 min.                   | 2 min.                   |    |
|    | Color of stock                 | Black                    | Black                    | Black                    | Black                    |    |
|    | Color of finished product      | Slightly improved.       | 6 N. P. A.               | 5 1/4 N.                 | 4 1/4 N. P. A.           |    |

the naphthenic acids containing the carbonaceous materials, or by treating the impure naphthenic acids with concentrated aqueous solutions of hydrogen halides. The function of any of the above reagents is to coagulate the carbonaceous materials to particles large enough to settle under the influence of gravity. I have discovered that naphthenic acids which have been freed from carbonaceous material by means of any of the above mentioned reagents are readily amenable to treatment with an adsorbent material in the manner described above.

While the process of deodorization and decolorization has been particularly described in connection with phenol-free or "semi-refined" naphthenic acids, it may equally well be applied to naphthenic acids which have not been subjected to a process for the removal of phenolic materials such as that previously described. However, such products do not possess as desirable a color and odor as the naphthenic acids which had been freed from phenolic material.

The term "blowing bright" referred to earlier in this specification, relates to the treatment of naphthenic acids or other hydrocarbon products with an inert gas, such as air or methane, ethane, and the like, for removing traces of water which remain in the naphthenic acids or other liquid hydrocarbon after a treatment thereof with water or aqueous solutions.

The term "Filtrol" signifies an acid treated clay or fuller's earth. The product commercially marketed under that name consists of fuller's earth which has been activated by means of dilute sulphuric acid.

The term "N. P. A. color" used in this specification relates to a color grade of a liquid obtained by means of the Union petroleum colorimeter adapted as a standard of the National Petroleum Association in 1915. A detailed description of the apparatus, method of test and significance of scale readings may be found in David T. Day's "Handbook of Petroleum Ind.", 1922, vol. 1, page 665. For example N. P. A. 0.5-1 indicates a light, almost water-white color, wherein N. P. A. 3 indicates a yellow to straw color and N. P. A. 7 to 8 indicates a product of a dark reddish to brown color.

The process herein set forth is applicable to all varieties of naphthenic acids. It may be equally well applied to naphthenic acids derived from a light petroleum fraction such as kerosene as to acids derived from the higher boiling fractions such as gas oil or lubricating oil.

The examples set forth herein are merely illustrative of the generic invention and many variations thereof will be obvious to those skilled in the art.

I claim:

1. A process for deodorizing and decolorizing crude naphthenic acids substantially free from carbonaceous materials which comprises treating said acids with an adsorbent material.

2. A process for deodorizing and decolorizing crude naphthenic acids substantially free from carbonaceous materials which comprises admixing said acids with an adsorbent material, heating the mixture of naphthenic acids and adsorbent material to a temperature in excess of normal room temperature and separating the spent adsorbent material from the naphthenic acids.

3. A process for deodorizing and decolorizing crude naphthenic acids which comprises contacting said acids with a reagent adapted to remove carbonaceous materials admixed with the said

naphthenic acids and contacting the so treated naphthenic acids with an adsorbent material.

4. A process for deodorizing and decolorizing crude naphthenic acids which comprises removing carbonaceous materials admixed with the said naphthenic acids and subsequently treating the said naphthenic acids with an adsorbent material at temperatures in excess of normal room temperature.

5. A process for deodorizing and decolorizing crude naphthenic acids which comprises contacting said acids with an oxygen-containing inorganic acid capable of removing carbonaceous materials admixed with the said naphthenic acids and contacting the so treated naphthenic acids with an adsorbent material at temperatures substantially in excess of normal room temperature.

6. A process for deodorizing and decolorizing crude naphthenic acids which comprises contacting said acids with sulphuric acid having a concentration between approximately 50 and 83% to remove carbonaceous materials admixed with the said naphthenic acids, and contacting the so treated naphthenic acids with an adsorbent material at temperatures substantially in excess of normal room temperature.

7. A process for deodorizing and decolorizing crude naphthenic acids which comprises contacting said acids with 80% sulphuric acid to remove carbonaceous materials admixed with the said naphthenic acids, and contacting the so treated naphthenic acids with an adsorbent material at temperatures substantially in excess of normal room temperature.

8. A process for deodorizing and decolorizing crude naphthenic acids which comprises contacting said acids with sulphuric acid having a concentration between approximately 83%  $H_2SO_4$  and about 15% dissolved  $SO_3$ , in the presence of a light hydrocarbon to obtain a naphthenic acid phase comprising naphthenic acids dissolved in said light hydrocarbon and a phase comprising acid sludge and carbonaceous materials originally admixed with the said naphthenic acids, separating the two phases and contacting the naphthenic acid phase with an adsorbent material at temperatures in excess of normal room temperature.

9. A process for deodorizing and decolorizing crude naphthenic acids which comprises contacting said acids with sulphuric acid having a concentration of approximately 95% in the presence of a light hydrocarbon to obtain a naphthenic acid phase comprising naphthenic acids dissolved in said light hydrocarbon and a phase comprising acid sludge and carbonaceous materials originally admixed with the said naphthenic acids, separating the two phases and contacting the naphthenic acid phase with an adsorbent material at temperatures in excess of normal room temperature.

10. A process for deodorizing and decolorizing crude naphthenic acids which comprises removing carbonaceous materials admixed with the said naphthenic acids and subsequently treating said naphthenic acids with an adsorbent material at temperatures which are below the boiling point of the said naphthenic acids.

11. A process for deodorizing and decolorizing crude naphthenic acids which comprises removing carbonaceous materials admixed with the said naphthenic acids and subsequently treating said naphthenic acids with an adsorbent material at temperatures ranging from approximately 225 to 325° F.

12. A process for deodorizing and decolorizing crude naphthenic acids which comprises removing carbonaceous materials admixed with the said naphthenic acids and subsequently treating 5 said naphthenic acids with an adsorbent material in the presence of an inorganic substance capable of liberating hydrogen ions, at temperatures substantially in excess of normal room temperature.
- 10 13. A process for deodorizing and decolorizing crude naphthenic acids which comprises removing carbonaceous materials admixed with the said naphthenic acids and subsequently treating 15 said naphthenic acids with an adsorbent material in the presence of an inorganic acid sulfate capable of liberating hydrogen ions at temperatures substantially in excess of normal room temperature.
14. A process according to claim 6 in which the 20 adsorbent used in fuller's earth which has been activated with sulphuric acid.
15. A process for deodorizing and decolorizing crude naphthenic acids which comprises contacting said acids with sulphuric acid, removing 25 sludge and carbonaceous materials which have been agglomerated due to the action of the sulphuric acid without removing the residual sulphuric acid remaining admixed with the naphthenic acids, contacting the naphthenic acids at 30 elevated temperatures with an adsorbent material in the presence of said residual sulphuric acid and separating the spent adsorbent material from the naphthenic acids.
- 35 16. A process according to claim 15 comprising the additional step of incorporating a small amount of water into the mixture of naphthenic acids, residual sulphuric acid and adsorbent material for the purpose of realizing a more efficient activation of the adsorbent material by the 40 residual sulphuric acid.
17. A process for deodorizing and decolorizing crude naphthenic acids which comprises contacting said acids with sulphuric acid having a concentration between approximately 50 and 83% 45 to remove carbonaceous materials admixed with the said naphthenic acids, removing acid sludge together with the carbonaceous materials from the naphthenic acids, water washing the naphthenic acids to remove residual sulphuric acid, blowing the naphthenic acids with an inert gas to remove the remaining traces of water and contacting the so treated naphthenic acids with
- an adsorbent material at temperatures substantially in excess of normal room temperature.
18. A process according to claim 17 in which the adsorbent used has been activated with an inorganic acid. 5
19. A process for deodorizing and decolorizing crude naphthenic acids which comprises contacting said acids with sulphuric acid having a concentration between approximately 50 and 83% at a temperature substantially in excess of normal room temperature, removing carbonaceous materials and acid sludge from the naphthenic acids and contacting the so treated naphthenic acids with an adsorbent material at temperatures substantially in excess of normal room temperature. 10 15
20. A process for deodorizing and decolorizing crude naphthenic acids which comprises contacting said acids with sulphuric acid having a concentration between approximately 83%  $H_2SO_4$  and about 15% dissolved  $SO_3$ , at a temperature substantially in excess of normal room temperature, removing carbonaceous materials and acid sludge from the naphthenic acids and contacting the so treated naphthenic acids with an adsorbent material at temperatures substantially in excess of normal room temperature. 25 20
21. A process for deodorizing and decolorizing crude naphthenic acids which comprises contacting said acids in the presence of a light hydrocarbon with a reagent adapted to remove carbonaceous materials admixed with the said naphthenic acids, separating a naphthenic acid phase comprising naphthenic acids dissolved in said light hydrocarbon from a phase comprising the aforesaid reagent and carbonaceous materials and treating the naphthenic acid phase with an adsorbent material at temperatures in excess of normal room temperature. 30 35
22. A process for deodorizing and decolorizing crude naphthenic acids which comprises contacting said acids with sulfuric acid having a concentration in excess of approximately 83%  $H_2SO_4$ , adding sulfuric acid of a concentration less than approximately 83%  $H_2SO_4$  to the mixture of naphthenic acids and sulfuric acid to obtain a naphthenic acid phase and a phase comprising acid sludge and carbonaceous materials, separating said phases and treating the naphthenic acid phase with an adsorbent material at 45 50 temperatures in excess of normal room temperature.

FREDERICK J. EWING.

CERTIFICATE OF CORRECTION.

atent No. 2,035,742.

March 31, 1936.

FREDERICK J. EWING.

It is hereby certified that error appears in the printed specification of the above numbered patent requiring correction as follows: Page 4, Table I, in next to last column thereof, last line, for "N." read N. P. A.; page 6, first column, line 20, claim 14, for "in" read is; and that the said Letters Patent should be read with these corrections therein that the same may conform to the record of the case in the Patent Office.

Signed and sealed this 2nd day of February, A. D. 1937.

Leslie Frazer

Seal)

Acting Commissioner of Patents.